

## UNITED STATES PATENT OFFICE

2,382,204

## CHROME TANNING SOLUTIONS AND METHOD OF MAKING AND USING THE SAME

Hiram B. Channon, Portsmouth, Va., assignor to  
 Virginia Smelting Company, West Norfolk, Va.,  
 a corporation of Maine

No Drawing. Application December 29, 1942,  
 Serial No. 470,470

4 Claims. (Cl. 8—94.26)

This invention relates to combination chrome tanning solutions and to the procedure of preparing and using the same.

In the preparation of tanning liquors for the tanning of leather by the procedures of chrome tanning as heretofore developed, it has been the common practice to use the aqueous solution of sodium or potassium dichromate which is reduced by the addition of sulphur dioxide or of sugar or like reducing agents.

Such reduction of dichromate is in general satisfactory, but it is susceptible to numerous conditions and variations and the resulting tanning liquor and its tanning activity vary accordingly. The concentrations of the several reagents, the rates and temperatures at which they are reacted, and their ultimate proportions are all important features. In all cases an excess of sugar is required to effect complete reduction of the dichromate, so that various by-products are formed. Moreover, too rapid a reaction will caramelize or carbonize a part of the sugar, which is detrimental to its use as a tanning agent, and the reducing reaction proceeds out of control, with unknown variations in the composition of the end products accordingly.

It is, therefore, an object of this invention to provide improved tanning solutions or liquors for the chrome tanning of leather which may be definitely prepared of reliable composition and which may be used in the tanning procedure with uniformity of operation and dependability of the results to be obtained. Other objects will appear from the following disclosure.

In accordance with the present invention it is discovered that a properly reduced chrome tanning liquor may be accurately and definitely prepared and that it will be effectively maintained in a proper condition for functioning dependably throughout the tanning operation by the preliminary addition thereto—before applying to the hides to be tanned—of certain characteristically strong organic acids.

Organic acids are in many cases too weakly acidic, though the relatively strong organic acids such as formic, oxalic and acetic acids are effective for the purpose of this invention, and more especially so when used in conjunction with each other in a given reduced chrome tanning liquor. A plurality of the organic acids may be employed, therefore, with advantageous results in getting a more complete and greatly improved tanning.

Chrome tanning liquors, as thus prepared, manifest a more uniform tanning action from the start and carry out automatically a more uniform

and complete tanning throughout the untanned hide and resulting leather than any of the usually reduced chrome tan liquors as known and used in the tanning art before the present invention, whether reduced from the dichromate by sulphur dioxide or by organic reducing agents such as sugar, organic wastes, etc. They are characterized by a combined tanning action upon the hides to which they are applied; which is chemically so controlled that it automatically avoids the variations in the operations and results which are above pointed out with respect to commercial tanning liquors of the prior art.

The combined tanning action of the ingredients of such treated liquors, containing the reduced chrome and the organic acid thus added in accordance with the present invention, is characterized by a gradual, uniform, progressive and complete permeation of the hide to a uniform concentration throughout, before the tanning action is effective to retard or prevent such permeation. Hence, as the tanning action proceeds, the hide is developed into leather as a whole, and the inner portions are tanned as well and as completely as the outer portions. Moreover, the fiber elements of the hide structure are individually penetrated and their lumens filled as well as the porous spaces and the hide substances which are between the fibers. This is an extremely important feature of the present invention. And yet it is secured without increased time being required for the tanning operation and without the necessity of expensive reagents or additional equipment.

It is thus discovered that by tanning hides with the combination tanning solutions as thus prepared an improved tanning operation or function is accomplished in the process and that a fundamental improvement in the tanning characteristics of the finished leather is obtained, as will be pointed out more fully below.

Moreover, if these conditions are observed, it is not necessary to reduce the dichromate with sugar. Therefore, the dichromate solution may be more definitely reduced with sulphur dioxide and then stabilized by the addition of the weakly acidic reagent, without introducing the variable by-products of the sugar reaction.

50

1

For example, in a given case, 100 lbs. of sodium dichromate were dissolved in 50 gallons of water and the resulting solution reduced by introducing 55 liquid sulphur dioxide therein gradually, in sub-

stantially theoretical proportion (64.5 lbs.) according to the reaction:



The solution which has been reduced as above described may be treated with one or more organic acids, so chosen and in such amounts as to give the resulting treated liquor a pH value between 2.8 and 3.0. For example, a mixture of 2% of oxalic acid, 1% formic acid and 1% acetic acid (calculated upon the weight of the original dichromate in the solution) was added to and dissolved in the solution (after the desired initial reduction has been completed) resulting in an especially suitable and satisfactory liquor for chrome tanning.

The solution, as thus prepared and in the quantities and concentrations indicated, was found to be satisfactory for direct use in the tanning of 1000 lbs. of hides, weighed after pickling and draining.

### II

In another mode of procedure 1000 lbs. of dichromate were dissolved in 250 gallons of water, 10 lbs. of acetic acid (100%) were added to the resulting solution, and liquid sulphur dioxide introduced gradually until the temperature reached 120° F. The sulphur dioxide stream was then shut off and 100 lbs. of caustic soda, dissolved in about 50 gallons of water, added. The stream of sulphur dioxide was then turned on and continued until reduction of the solution was complete. Then added 10 lbs. formic acid (100%) and 20 lbs. of oxalic acid (100%). Agitation was continued till the additions were thoroughly dissolved and the volume increased by additions of water to provide a concentration corresponding to 2 lbs. of original dichromate to the gallon, or 500 gallons total final volume.

The addition of the acetic acid tends to give a bluish cast to the chrome, but does not take part in the reduction. It could be added last, i. e., with the oxalic and formic acids if desired.

It is to be observed that in the combination tanning liquors as thus prepared the weakly acid reagent, whether provided in the form of a strong organic acid or acids such as acetic formic and oxalic acids combined, is present in a molecular ratio with respect to the sodium dichromate from which the tanning liquor has been prepared of one-sixth to one-third. Lesser proportions of the acidic reagent are in general ineffective while larger proportions are characterized by a tendency to convert the chrome content of the liquor from the green form or modification to the violet or reddish modification, which is not susceptible of control of the tanning action as herein discovered, disclosed and claimed.

The combined tannage action of the chrome liquor as thus modified by the acidic reagent is different both in kind and in degree from chrome tan liquors of the prior art, and also in respect of the tanning function and of the tanned leather product obtained, as will be pointed out and discussed below.

In the tanning procedure with such chrome tannage liquors, 1000 lbs. of stock may be taken, after pickling and draining, and laid down with 100 gallons of water in which 40 lbs. of common salt have been dissolved. The charge as thus prepared is handled in a wheel or rotatable drum, to which the reduced dichromate solution, as obtained by any of the procedures above described, is added. Thus, a total quantity of re-

duced chrome solution, under I, corresponding to 40 lbs. of dichromate (in a concentration of 2 lbs. to the gallon and hence equal to 20 gallons) are diluted with water to 30 gallons. Thus, for example, on the weight of the dichromate it may contain

|             | Per cent |
|-------------|----------|
| Oxalic acid | 2 to 4   |
| Formic acid | 1 to 2   |
| Acetic acid | 1 to 2   |

and complete solution of all of the reagents is effected.

This solution is then added to the wheel in 4 equal portions, one hour apart, and the drumming of the hides continued for 3 hours thereafter.

Then 1 1/4% sodium bicarbonate (on the weight of the stock) is dissolved in water to a concentration of 1/4 lb. per gallon (or 12 1/2 lbs. of bicarbonate in 50 gallons of solution) and this is added to the hides in two equal portions, 15 minutes apart.

The charge is then drummed for 1/2 hour longer. The drumming is stopped and the charge allowed to lie quiescent over night. The next morning the charge is drummed for 1/2 hour and the contents are discharged. The stock is hosed up and allowed to drain.

The leather thus obtained is more especially suitable for use as upper leather. In making leather for other purposes, the manipulation, concentration, periods of treatment and amounts of the acidic reagent present and of the sodium bicarbonate subsequently added will be adapted accordingly, in ways known to or readily determinable by those skilled in the art from the above description and examples.

It is also found that acid solutions of dichromate or chromic acid solutions which have been reduced with sugar or other organic reducing agents while undergoing indeterminate amounts of side reactions and containing variable amounts of by-products accordingly may be treated by the addition of the above described strong organic acid reagents thereto, in accordance with the invention.

During the latter part of the tanning action the pH value of the tanning liquor usually rises from about 3.0 to 4.6. But during the preliminary part of the tanning action the pH value of the combination tanning liquor prepared as herein described is such as to serve the double function of keeping the tanning agents in solution and of definitely promoting its penetration and permeation of the several structures of the leather substance as a whole and more especially of the individual fibers, as will be described below.

It is found that leathers tanned by the present invention have a modified feel and resiliency in contrast to those obtained by a chrome tanning liquor reduced by mineral reducing agents only. Moreover, whereas ordinary pickled stock shows a tendency to curl at 55° C., the products obtained as above described may be boiled without curling. These products are full and resilient, giving the body and resistance to bending and folding which is so desirable in well tanned leathers.

This quality is sometimes tested for by folding the leather tightly and then advancing one fold over the other and noting whether it squeaks. This test is believed to indicate whether the capillaries of the leather have been penetrated by the tanning solution.

It is well known that the spaces in the in-

dividual fibers, or lumens, in their normal functions in the hide of the living animal contain various circulating tissue fluids such as lymph, etc. There is, accordingly, an interchange of fluids through the cell walls of these lumens and discharge of metabolized products back from the lumens into the lymphatic system, for example. In the various treatments to which hides are subjected, the tissue fluids contained in the lumens of the fibers are substantially removed, thus leaving the hollow fibers filled with water only and upon its removal, as by drying, the fibers collapse and the hide as a whole loses its resiliency and is either stiff and hard when dry or soft and flaccid if moist.

In tanning hides, therefore, it is desirable to impart resiliency to these individual fibers, as such, as well as to the spaces or materials between them. This is not effected by chrome tanning liquors and processes of the prior art. In order to do so the interior portions of the lumens of the individual fibers must be treated, at least partially, with the tanning liquor. To accomplish this result, it is necessary for the tanning solution to permeate both the leather structure and the walls of the individual fibers, and thus enter the lumens laterally throughout their length as well as to enter the lumens at their ends or other openings, and thus penetrate them longitudinally from one end to the other, by osmosis and capillarity.

It is found that the combination dichromate tanning solutions which have been prepared as above described are effective not only to pass through the general structure of the hide interly but also to penetrate the walls into the lumens of the individual fibers intrally, and even to permeate the walls of such individual fibers, and thus to enter the lumens of such fibers and to fill both the lumens and the fiber walls with the tanning solution. This noticeably expands and plumps out each individual fiber in the leather. In the tanning action, effected by the present invention, the hydrated chromium component of the impregnating liquor is separated out and being already within the lumens precipitates upon the inner walls of the lumens of the fibers and thus fills or at least coats and partially fills them with an initially gelatinous precipitate which may, upon subsequent extreme drying, as in old leather objects made therefrom, be reduced to a finely divided powder. In the gelatinous form it retains the lumens in moist, expanded condition, and gives the leather a fullness and firmness of texture, or body, which is an extremely desirable quality. The fibers, as thus individually filled out by the gelatinous precipitate in the lumen of each one, are more resistant to folding and also exert their elasticity more effectively to resume their original shape and position after folding, than a collapsed and stiffened fiber can do. They, therefore, impart resiliency and life to the leather as a whole. Moreover, since they are to an appreciable degree kept moist by the gelatinous precipitate thus deposited in them, such fibers remain pliable longer than would otherwise be the case. And if and when they may ultimately dry out and lose their moisture, the residual finely divided chromium hydroxide or oxide, which is then left, lubricates the opposite walls of the lumen, one from the other, and keeps them apart. The

fibers are therefore relieved, by the more or less filled inner structure of the lumens, when the leather is folded, so that the fibers are not so sharply folded and creased as they would be if the lumens were collapsed and the inner surfaces were either adherent to each other or frictionally in contact with each other.

The result of tanning hides with the combination chrome tanning solutions prepared in accordance with the present invention is that the fibers are individually tanned on the inside and plumped. Therefore, they are more flexible and also more resilient to return to their natural shape and disposition, and hence produce leather of greater body and fullness than is obtained by tanning liquors which are prepared in accordance with the prior art and practices.

This application is a continuation-in-part of my copending application Serial No. 264,189, filed March 25, 1939.

I claim:

1. A combination chrome tannage for hides, comprising the steps of treating a sulphur dioxide reduced dichromate tanning liquor with an organic acid selected from the group consisting of oxalic, formic and acetic acids and mixtures thereof, in a total molecular proportion of one-sixth to one-third of the dichromate to a pH value between approximately 2.8 and 3.0, and then applying the resulting liquor to the hides to be tanned, whereupon the liquor plumps the hides and penetrates the fiber structure and lumens of the hides, preliminary to the tanning action thereof.

2. A chrome tanning liquor consisting substantially of a solution of mono-basic chromic sulphate, and an organic acid selected from the group consisting of oxalic, formic and acetic acids and mixtures thereof in the molecular ratio of approximately one-sixth to one-third of the mono-basic chromic sulphate present, having a pH value between 2.8 and 3.0 whereby, upon contact with pickled hides, the liquor plumps the hides and penetrates the fiber structure and lumens thereof, preliminary to the tanning action.

3. Method of preparing a combination chrome tanning liquor, preliminary to the operation of tanning pickled and drained hides therewith, comprising the steps of reducing an aqueous solution of an alkali metal dichromate with sulphur dioxide, while maintained in acidic condition, completely to the form of mono-basic chromic sulphate, and then treating the latter with an organic acid selected from the group consisting of oxalic, formic and acetic acids and mixtures thereof in the molecular proportion of approximately one-sixth to one-third of the dichromate to a pH value between approximately 2.8 and 3.0, whereby, upon contact with the pickled and drained hides, the liquor plumps the hides and penetrates the fibrous structure and the lumens of the hides, preliminary to its tanning action thereof.

4. The method of tanning hides which comprises applying the tanning liquor of claim 2 to the hides, in pickled and drained condition, and initially plumping the hides by reason of contact with said liquor whereby the tanning liquor penetrates the hides preliminary to the tanning action.

HIRAM B. CHANNON.